# EUROPEAN PATENT SPECIFICATION

(11) **EP 2 071 965 B1**
(45) Date of publication and mention of the grant of the patent: **17.11.2010**
(21) Application number: 07400034.0
(22) Date of filing: 20.12.2007
(51) Int. Cl.: A24C 5/00, A24D 1/02, A24C 5/46, D21H 17/66, D21H 23/22, A24C 5/40, A24D 1/10

(54) **Smoking article with improved extinguishing characteristics**
Rauchware mit verbesserten Auslöscheigenschaften
Article à fumer avec des caractéristiques d'extinction améliorées

(43) Date of publication of application: 24.06.2009
(73) Proprietor: Reemtsma Cigarettenfabriken GmbH, 22761 Hamburg (DE)
(72) Inventor: Pienemann, Thomas, DE 21224 Rosengarten (DE)
(74) Representative: Both, Georg

(56) References cited:
- EP-A- 0 314 138
- EP-A- 0 333 506
- EP-A- 0 981 971
- EP-A- 1 234 514
- EP-A- 1 867 782
- EP-B- 0 999 937
- WO-A-96/35841
- KR-A- 20040 027 557
- US-A- 2 775 970
- US-A- 4 183 362
- US-A- 4 453 553
- US-A- 5 048 546
- US-A1- 2006 021 625
- US-B1- 6 783 847
- [Online] XP002502040 Retrieved from the Internet: URL:http://www.handpapermaking.org/Sizing. html> [retrieved on 2008-10-30]

## Description

The invention relates to a smoking article (claim 1) with improved extinguishing characteristics (reduced or lower ignition propensity or ignition proclivity), to a method of manufacturing such a smoking article (claim 10), to a wrapper (claim 15) and to a wrapper tube (claim 16).

Product regulations in many countries specify that cigarettes have to fulfil certain safety standards regarding their ignition propensity. The ignition propensity of cigarettes can be measured by a standardized test method. Usually, the test defined in ASTM E 2187-04 is performed (ASTM: "American Standard for Testing and Materials"; ASTM E 2187: "Standard Test Method for Measuring the Ignition Strength of Cigarettes"; the extension "-04" refers to 2004 as the year of the last revision). According to ASTM E 2187-04, a sample of 40 cigarettes is tested under well-defined conditions, and the fraction of these cigarettes which burn their full length is called "the test result". A safety standard specifies which test result is acceptable. For example, in Canada and some U.S. states, the acceptable test result is 25%, i.e. at least 75% of the cigarettes have to extinguish before burning their full length in order to comply with the safety standard.

The most common way to reduce the ignition propensity of cigarettes is to enhance the extinguishing characteristics by using a paper wrapper comprising spaced bands of lower porosity, which extend along the circumference of the wrapper. By these means, oxygen supply is reduced when the burning cone of the cigarette reaches a respective band, and the cigarette extinguishes when smoldering on a substrate, as described in ASTM E 2187-04. Common methods to produce such banded cigarette papers are described in EP 1 234 514 A2.

A general disadvantage of using low-porosity bands on wrapper papers is a reduced rod ventilation caused by the reduced porosity in these bands, resulting in changes of CO/NFDPM ratios to often undesired levels (CO: carbon monoxide, NFDPM: nicotin-free dry particulate matter).

The use of inorganic salts as burn retardants is commonly known, including some applications for tobacco products. Inorganic salts as such, however, have not been used for reducing ignition propensity, which is probably based on the assumption that a certain oxygen deficit is necessary to make cigarettes self-extinguish in the ASTM test cited above and that this can only be achieved by reducing the wrapper porosity to a level lower than 10 CU to 15 CU (CU: Coresta unit, permeability as measured in the tobacco industry, see CORESTA Recommend Method No. 40). In EP 1 234 514 A2, disclosing the features of the preamble of claim 1, e.g., ammonium phosphate is used as a burn retardant, but only in combination with additional substances, as e.g. alginates, which provide for a low porosity.

The object of the invention is to provide a smoking article with reduced ignition propensity, which does not exhibit the disadvantage of a significantly reduced rod ventilation.

This object is achieved by a smoking article having the features of claim 1. Claim 10 relates to a method of manufacturing such an article. Claims 15 and 16 relate to a wrapper for rolling cigarettes and to a wrapper tube for making cigarettes, respectively, which have a reduced ignition propensity. Advantageous embodiments of the invention emerge from the dependent claims.

The smoking article according to the invention comprises a tobacco rod and a wrapper. The wrapper includes at least one zone treated with an inorganic salt providing reduced ignition propensity. This zone can comprise the total wrapper. In advantageous embodiments of the invention, however, the wrapper includes at least one discrete zone treated with the inorganic salt, wherein the total surface area of the discrete zones is smaller than the total surface area of the wrapper; i.e. in addition to any areas of the wrapper being covered by, e.g., a tipping paper of a filter, there are exposed areas of the wrapper which are not treated with the inorganic salt.

Surprisingly, it was found that the application of inorganic salts is able to reduce the ignition propensity of the smoking article without reducing the porosity of the wrapper to levels as commonly required for this purpose. Thus, the invention does not rely on the main effect of a reduced porosity in the zones treated with the inorganic salt.

According to the invention, the porosity of the wrapper in the treated zones is larger than 10 CU, preferably larger than 12 CU or than 15 CU. Porosities in this range permit access of sufficient oxygen to the tobacco rod in order to minimise carbon monoxide formation and provide for sufficient diffusion.

The inorganic salt can comprise, e.g., magnesium chloride, aluminium sulfate, alum, sodium tetraborate, hydrated magnesium chloride, hydrated aluminium sulfate, hydrated alum, hydrated sodium tetraborate, sodium chloride, or mixtures thereof. In the discrete zones of the wrapper, the specific amount of the organic salt can be in the range of from 0.2 mg/cm² to 20 mg/cm² or in the range of from 0.5 mg/cm² to 5 mg/cm². Moreover, any interval limits in the range of from 0.2 mg/cm² to 20 mg/cm² are explicitly disclosed herewith. Such inorganic salts are less expensive than porosity-reducing agents like alginates.

In advantageous embodiments of the invention, there are discrete zones treated with the salt(s) arranged as bands (rings) extending along the circumference of the smoking article and having a width, measured along the tobacco rod axis, of from 2 mm to 12 mm or from 2 mm to 8 mm or preferably of 6 mm. Generally, the provision of the inorganic salts in the bands is sufficient for achieving reduced ignition propensity such that it is not required to treat the whole wrapper material with the inorganic salt, which results, e.g., in cost reduction and the possibility of an even higher porosity in the wrapper areas between the discrete zones. Preferably, the wrapper comprises at least two such bands which are separated by at least 1 mm or at least 5 mm and preferably by at least 10 mm.

In advantageous embodiments of the invention, the smoking article comprises a filter, and the smoking article can be designed as a cigarette, wherein the wrapper is a cigarette paper (which includes the possibility of manufacturing the wrapper from reconstituted tobacco).

Other embodiments of the invention relate to a wrapper for rolling cigarettes (RYO cigarettes; RYO: "Roll Your Own"), as well as to a wrapper tube (preferably a paper tube including a filter at one of its ends) for making cigarettes (MYO cigarettes; MYO: "Make Your Own") by filling the paper tube with tobacco. In these cases, the wrapper paper and the wrapper tube comprise, with respect to reduced ignition propensity, the features of the wrapper of a smoking article explained so far.

There are several ways of manufacturing a smoking article according to the invention, in particular of applying the inorganic salts to the wrapper. These methods can be applied to a paper for rolling cigarettes or to a paper tube for making cigarettes in an analogue way.

In advantageous embodiments, the inorganic salt is applied to the wrapper by means of a solution or suspension. To improve the solubility of the inorganic salt, such solution can be heated. Preferably, the solvent or the suspension agent comprise water.

The inorganic salt can be applied to the wrapper by, e.g., printing techniques like gravure printing or inkjet printing, but also techniques like spraying or sizing. Printing techniques are very precise and can even be used online, e.g., in a cigarette making process after wrapping a continuous tobacco rod with the wrapper material.

For example, the inorganic salt can be applied to the wrapper by sizing in a papermaking process for providing the material of the wrapper. Whereas, usually, sizing is applied to the overall surface of the paper produced in a papermaking process, it is also possible to size zones of the paper only.

In another possibility, the inorganic salt is applied to the wrapper immediately after a papermaking process during the cutting step of a mother reel into bobbins containing wrapper material, as usually performed in the cigarette paper industry in order to provide wrapper material suitable for use in a cigarette making machine.

When a bobbin containing ordinary wrapper material is provided, the inorganic salt can be applied to the wrapper material during a rewinding step of such bobbin. This step is performed offline, i.e. not during the usual operating steps of a cigarette making machine.

It is also possible to apply the inorganic salt to the wrapper during a cigarette making process, i.e. online, either before wrapping a continuous tobacco rod with the wrapper material or after wrapping a continuous tobacco rod with the wrapper material. For such applications, gravure printing and inkjet printing, which apply a solution or suspension of the inorganic salt as "ink", are particularly suitable.

In the following, the invention is described in more detail by means of several embodiments, which are not considered as exclusive.

### Example A

In a pilot test, cigarette papers were homogeneously treated with inorganic salts according to the invention, and the porosity of the respective cigarette paper was measured before the treatment and after the treatment. The porosity measurements were performed according to CORESTA Recommended Method No. 40. 1 CU ("CORESTA unit") is the air flow (in cm³/min) through an area of the cigarette paper of 1 cm² when the pressure difference across the cigarette paper is 1 kPa. The following table shows the initial porosity ("base porosity") of the cigarette paper, the salt and its amount applied as well as the porosity after the salt treatment ("remaining porosity").

| Base porosity | Salt | Amount | Remaining porosity |
|---|---|---|---|
| 35 CU | Magnesium chloride (hydrate) | 1.2 mg/cm² | 16 CU |
| 35 CU | Aluminium sulfate (hydrate) | 3.0 mg/cm² | 11 CU |
| 35 CU | Sodium chloride | 4.0 mg/cm² | 64 CU |
| 50 CU | Aluminium sulfate (hydrate) | 3.0 mg/cm² | 18 CU |

It is evident that the remaining porosity is larger than 10 CU in all cases and significantly larger than 10 CU in most of the cases.

### Example B

In another test, a commercial cigarette comprising a cigarette paper with a base porosity of 35 CU was homogeneously treated with an aqueous solution of sodium chloride until a weight of 4.0 mg sodium chloride per cm² was achieved.

The test result according to ASTM E 2187-04 (see above) for cigarettes treated in this way was 35%.

### Example C

The outer side ("felt side") of a commercial cigarette paper (base porosity 35 CU) was sprayed with an aqueous solution of magnesium chloride to form treated discrete zones in band form of 6 mm width with a distance (gap width) of 20 mm on the paper. The concentration of the solution and the amount of spraying were adjusted so that a weight of 1.2 mg magnesium chloride per cm² was achieved. In other embodiments, the inner side ("wire side") or both sides of the cigarette paper could be sprayed with the solution.

Conventional American Blend cigarettes were produced with the treated paper and tested according to ASTM E 2187-04. The test result was 13%.

### Example D

A warm (50°C), saturated solution of aluminium sulfate was applied to the cigarette paper (porosity 50 CU) of a conventional cigarette during the cigarette making process using a gravure printing device. The gravure depth was adjusted so that a weight of 3 mg aluminium sulfate per cm² was achieved in the printed areas. The salt was applied in band-shaped discrete zones having a width of 6 mm each and a respective distance (width of untreated zones) of 20 mm.

According to ASTM E 2187-04, the test result was 20%.

## Claims

1. Smoking article, comprising a tobacco rod and a wrapper, wherein the wrapper includes at least one zone treated with an inorganic salt providing reduced ignition propensity, **characterized in that** the porosity of the wrapper in the treated zone(s), as a result of said treatment, remains larger than 10 CU.

2. Smoking article according to claim 1, **characterized in that** the porosity of the wrapper in the treated zone(s) is larger than 12 CU or 15 CU.

3. Smoking article according to claim 1 or 2, **characterized in that** the inorganic salt comprises at least one substance selected from the group consisting of magnesium chloride, aluminium sulfate, alum, sodium tetraborate, hydrated magnesium chloride, hydrated aluminium sulfate, hydrated alum, hydrated sodium tetraborate, sodium chloride.

4. Smoking article according to anyone of claims 1 to 3, **characterized in that** the specific amount of the inorganic salt in the treated zone(s) of the wrapper is in the range of from 0.2 mg/cm² to 20 mg/cm², preferably in the range of from 0.5 mg/cm² to 5 mg/cm².

5. Smoking article according to anyone of claims 1 to 4, **characterized in that** the wrapper includes at least one discrete zone treated with the inorganic salt, wherein the total surface area of the discrete zones is smaller than the total surface area of the wrapper.

6. Smoking article according to claim 5, **characterized in that** the discrete zones are arranged as bands extending along the circumference of the smoking article and having a width, measured along the tobacco rod axis, of from 2 mm to 12 mm, preferably of from 2 mm to 8 mm, most preferred of 6 mm.

7. Smoking article according to claim 6, **characterized in that** the wrapper comprises at least two discrete zones, two neighboring discrete zones being separated by at least 1 mm, preferably by at least 10 mm.

8. Smoking article according to anyone of claims 1 to 7, **characterized in that** it comprises a filter.

9. Smoking article according to anyone of claims 1 to 8, **characterized in that** it is a cigarette, the wrapper being a cigarette paper.

10. Method of manufacturing a smoking article according to anyone of claims 1 to 9, which includes a step being **characterized in that** the inorganic salt is applied to the wrapper by means of a solution or a suspension.

11. Method according to claim 10, **characterized in that** the solution is heated to improve the solubility of the inorganic salt.

12. Method according to claim 10 or 11, **characterized in that** the solvent or suspension agent, respectively, comprises water.

13. Method according to anyone of claims 10 to 12, **characterized in that** the inorganic salt is applied to the wrapper by one of the following techniques: gravure printing, inkjet printing, spraying.

14. Method according to anyone of claims 10 to 13, **characterized in that** the inorganic salt is applied to the wrapper online in a cigarette making process, before wrapping a continuous tobacco rod with the wrapper material.

15. Wrapper for rolling cigarettes, wherein the wrapper comprises the features of the wrapper of a smoking article according to anyone of claims 1 to 9 and wherein the wrapper is designed as a paper.

16. Wrapper tube, preferably including a filter, for making cigarettes by filling the wrapper tube with tobacco, wherein the wrapper tube comprises the features of the wrapper of a smoking article according to anyone of claims 1 to 9 and wherein the wrapper tube is designed as a paper tube.

## Patentansprüche

1. Rauchartikel, mit einem Tabakstab und einer Umhüllung, wobei die Umhüllung wenigstens eine mit einem anorganischen Salz behandelte Zone aufweist, die eine verminderte Zündneigung bereitstellt, **dadurch gekennzeichnet, dass** die Porosität der Umhüllung in der/den behandelten Zone/Zonen als Resultat dieser Behandlung größer als 10 CU bleibt.

2. Rauchartikel nach Anspruch 1, **dadurch gekennzeichnet, dass** die Porosität der Umhüllung in der/den behandelten Zone/Zonen größer als 12 CU oder 15 CU ist.

3. Rauchartikel nach Anspruch 1 oder 2, **dadurch gekennzeichnet, dass** das anorganische Salz wenigstens eine Substanz aufweist, die ausgewählt ist aus der Gruppe bestehend aus Magnesiumchlorid, Aluminiumsulfat, Alaun, Natriumtetraborat, hydratisiertem Magnesiumchlorid, hydratisiertem Aluminiumsulfat, hydratisiertem Alaun, hydratisiertem Natriumtetraborat, Natriumchlorid.

4. Rauchartikel nach einem der Ansprüche 1 bis 3, **dadurch gekennzeichnet, dass** die spezifische Menge des anorganischen Salzes in der/den behandelten Zone/Zonen der Umhüllung im Bereich von 0,2 mg/cm² bis 20 mg/cm² liegt, vorzugsweise im Bereich von 0,5 mg/cm² bis 5 mg/cm².

5. Rauchartikel nach einem der Ansprüche 1 bis 4, **dadurch gekennzeichnet, dass** die Umhüllung wenigstens eine mit dem anorganischen Salz behandelte diskrete Zone aufweist, wobei die gesamte Oberfläche der diskreten Zonen kleiner ist als die gesamte Oberfläche der Umhüllung.

6. Rauchartikel nach Anspruch 5, **dadurch gekennzeichnet, dass** die diskreten Zonen in Bändern angeordnet sind, die sich entlang des Umfangs des Rauchartikels erstrecken und eine entlang der Achse des Tabakstabs gemessene Breite von 2 mm bis 12 mm haben, vorzugsweise von 2 mm bis 8 mm, besonders bevorzugt von 6 mm.

7. Rauchartikel nach Anspruch 6, **dadurch gekennzeichnet, dass** die Umhüllung wenigstens zwei diskrete Zonen aufweist, wobei zwei benachbarte diskrete Zonen um wenigstens 1 mm getrennt sind, vorzugsweise um wenigstens 10 mm.

8. Rauchartikel nach einem der Ansprüche 1 bis 7, **dadurch gekennzeichnet, dass** er einen Filter aufweist.

9. Rauchartikel nach einem der Ansprüche 1 bis 8, **dadurch gekennzeichnet, dass** er eine Cigarette ist, wobei die Umhüllung ein Cigarettenpapier ist.

10. Verfahren zum Herstellen eines Rauchartikels nach einem der Ansprüche 1 bis 9, das einen Schritt aufweist, der **dadurch gekennzeichnet ist, dass** das anorganische Salz mittels einer Lösung oder einer Suspension auf die Umhüllung aufgetragen wird.

11. Verfahren nach Anspruch 10, **dadurch gekennzeichnet, dass** die Lösung erwärmt wird, um die Löslichkeit des anorganischen Salzes zu verbessern.

12. Verfahren nach Anspruch 10 oder 11, **dadurch gekennzeichnet, dass** das Lösungsmittel bzw. das Suspensionsmittel Wasser aufweist.

13. Verfahren nach einem der Ansprüche 10 bis 12, **dadurch gekennzeichnet, dass** das anorganische Salz durch eine der folgenden Techniken auf die Umhüllung aufgetragen wird: Tiefdruck, Tintenstrahldruck, Sprühen.

14. Verfahren nach einem der Ansprüche 10 bis 13, **dadurch gekennzeichnet, dass** das anorganische Salz in einem Cigarettenherstellungsverfahren online auf die Umhüllung aufgetragen wird, bevor ein fortlaufender Tabakstrang mit dem Umhüllungsmaterial umhüllt wird.

15. Umhüllung zum Rollen von Cigaretten, wobei die Umhüllung die Merkmale der Umhüllung eines Rauchartikels nach einem der Ansprüche 1 bis 9 aufweist und wobei die Umhüllung als ein Papier gestaltet ist.

16. Umhüllungsröhrchen, vorzugsweise mit einem Filter, zum Erstellen von Cigaretten durch Füllen des Umhüllungsröhrchens mit Tabak, wobei das Umhüllungsröhrchen die Merkmale der Umhüllung eines Rauchartikels nach einem der Ansprüche 1 bis 9 aufweist und wobei das Umhüllungsröhrchen als ein Papierröhrchen gestaltet ist.

## Revendications

1. Article à fumer, comprenant un boudin de tabac et une enveloppe, dans lequel l'enveloppe comporte au moins une zone traitée avec un sel inorganique assurant une tendance réduite à l'inflammation, **caractérisé en ce que** la porosité de l'enveloppe dans la/les zones traitées, par suite dudit traitement, reste supérieure à 10 unités Coresta CU.

2. Article à fumer selon la revendication 1, **caractérisé en ce que** la porosité de l'enveloppe dans la/les zones traitées est supérieure à 12 CU ou 15 CU.

3. Article à fumer selon la revendication 1 ou la revendication 2, **caractérisé en ce que** le sel inorganique est composé d'au moins une substance choisie dans le groupe comprenant le chlorure de magnésium, le sulfate d'aluminium, l'alun, le tétraborate de sodium, le chlorure de magnésium hydraté, le sulfate d'aluminium hydraté, l'alun hydraté, le tétraborate de sodium hydraté, le chlorure de sodium.

4. Article à fumer selon l'une quelconque des revendications 1 à 3, **caractérisé en ce que** la quantité spécifique du sel inorganique dans la/les zones traitées de l'enveloppe est de 0,2 mg/cm² à 20 mg/cm², de préférence de 0,5 mg/cm² à 5 mg/cm²,

5. Article à fumer selon l'une quelconque des revendications 1 à 4, **caractérisé en ce que** l'enveloppe comporte au moins une zone discrète traitée avec le sel inorganique, la superficie totale des zones discrètes étant plus petite que la superficie totale de l'enveloppe.

6. Article à fumer selon la revendication 5, **caractérisé en ce que** les zones discrètes sont organisées en bandes s'étendant sur le pourtour de l'article à fumer et ayant une largeur, mesurée sur l'axe du boudin de tabac, de 2 mm à 12 mm, de préférence de 2 mm à 8 mm, de préférence surtout de 6 mm.

7. Article à fumer selon la revendication 6, **caractérisé en ce que** l'enveloppe comporte au moins deux zones discrètes, deux zones discrètes voisines étant séparées d'au moins 1 mm, de préférence d'au moins 10 mm.

8. Article à fumer selon l'une quelconque des revendications 1 à 7, **caractérisé en ce qu'**il comprend un filtre.

9. Article à fumer selon l'une quelconque des revendications 1 à 8, **caractérisé en ce qu'**il s'agit d'une cigarette, l'enveloppe étant du papier à cigarettes.

10. Procédé de fabrication d'un article à fumer selon l'une quelconque des revendications 1 à 9, comprenant une étape **caractérisée en ce que** le sel organique est appliqué sur l'enveloppe à l'aide d'une solution ou d'une suspension.

11. Procédé selon la revendication 10, **caractérisé en ce que** la solution est chauffée afin d'améliorer la solubilité du sel organique.

12. Procédé selon la revendication 10 ou 11, **caractérisé en ce que** le solvant ou l'agent de suspension, respectivement, est composé d'eau.

13. Procédé selon l'une quelconque des revendications 10 à 12, **caractérisé en ce que** le sel inorganique est appliqué sur l'enveloppe à l'aide d'une des techniques suivantes : impression hélio, impression par jet d'encre, pulvérisation.

14. Procédé selon l'une quelconque des revendications 10 à 13, **caractérisé en ce que** le sel inorganique est appliqué en continu sur l'enveloppe durant un processus de fabrication de cigarettes, avant l'enveloppement d'un boudin de tabac continu avec le matériau enveloppant.

15. Enveloppe pour rouler des cigarettes, l'enveloppe comportant les caractéristiques de l'enveloppe d'un article à fumer selon l'une quelconque des revendications 1 à 9, l'enveloppe se présentant sous la forme de papier.

16. Tube enveloppant, comprenant de préférence un filtre, pour fabriquer des cigarettes en remplissant de tabac le tube enveloppant, le tube enveloppant comportant les caractéristiques de l'enveloppe d'article à fumer selon l'une quelconque des revendications 1 à 9, et le tube enveloppant se présentant sous la forme d'un tube en papier.
